

No. 682,991.

Patented Sept. 17, 1901.

T. H. MACDONALD.

PROCESS OF MAKING SOUND RECORDS.

(Application filed Nov. 3, 1900.)

(No Model.)



Fig. 2.



Fig. 1.

Fig. 3.



Witnesses

W. R. Edelen.

*George T. Tandy*

Inventor

Thomas H. Macdonald

*by Philip Mauro*  
*his Atty.*

# UNITED STATES PATENT OFFICE

THOMAS H. MACDONALD, OF BRIDGEPORT, CONNECTICUT.

## PROCESS OF MAKING SOUND-RECORDS.

SPECIFICATION forming part of Letters Patent No. 682,991, dated September 17, 1901.

Application filed November 3, 1900. Serial No. 35,351. (No model.)

*To all whom it may concern:*

Be it known that I, THOMAS H. MACDONALD, a citizen of the United States, and a resident of Bridgeport, Connecticut, have invented a new and useful Process of Making Sound-Records, which is fully set forth in the following specification.

This invention relates to improvements in sound-records and in the method of producing them by molding; and it consists in first superheating the material while in the mold and in then suddenly applying cold, whereby I obtain better results than heretofore possible.

15 The invention consists, further, in certain details to be hereinafter pointed out.

In order to explain my invention more readily, I refer to the annexed drawings, which show one form of apparatus for carrying out 20 my process.

Figure 1 is a vertical sectional view; and Fig. 2 is a plan, partly broken away. Fig. 3 is intended to illustrate the improved sound-record.

25 The record is cast into a suitable mold, which is surrounded by a steam and water jacket for superheating and cooling the casting. This jacket consists of an outer shell A and an inner shell B for the mold, these shells 30 inclosing between them the steam-tight space C. Shell A is closed at the bottom and open at the top for receiving shell B and is provided with valve-controlled inlets 1 and 2 for steam and cold water, respectively. Shell B

35 consists of a hollow cylinder B', also closed at the bottom b and open at the top, and has an annular flange B'', that rests upon the top of shell A and is secured thereto, as by screw-threaded lip b''. Flange B'' constitutes the

40 cover of the inclosed space C and serves to suspend shell B therein and is provided with the valve-controlled outlet 3. Core D has the base d fitting snugly in shell B' and resting on bottom b and at its upper end carries

45 the stem d'. A suitable matrix E is fitted snugly into shell B to rest upon base d. A head F is inserted in the top of shell B and rests squarely upon the top of matrix E and core D, stems d' taking into a suitable opening

50 in the head, which thus assists in securing the core in proper position. The annular space between the matrix and the core (con-

stituting the mold) is thus inclosed by the base d and the head F. The head is provided with the funnel 4, forming an inlet for pouring into the mold the melted material that is to form the improved sound-record.

55 In carrying out my invention I proceed as follows: I fill the mold (through funnel 4) with the melted material, (soap mixture or the like,) which is hereinafter, for convenience, designated "wax," though I do not limit myself to a wax-like composition, since any suitable material or composition that can be readily handled may be employed and will 60 come within the scope of my invention. I then admit steam through inlet 1 into the space C and heat the mold and its contents up to, say, about 350° centigrade and maintain the heat for some time, preferably until 65 the entire mass of the wax is in a limpid state. This superheating forces out all air-bubbles from the mass of the wax and from the minute spaces in and around the irregularities in the matrix-surface, thus producing a more 70 intimate relation between the molten wax and the matrix. After maintaining this heat 75 for a length of time sufficient to drive off all bubbles and impurities I then admit cold water through inlet 2 and allow the steam to escape through outlet 3. This sudden application of cold chills the surface of the wax 80 instantly and symmetrically and causes it to contract from the matrix-surface sufficiently to clear the now-solidified casting from the 85 matrix and permit its withdrawal. The fact that the cold acts evenly from all sides causes the contracting to be even and regular, so that cracking, &c., are avoided. Moreover, owing to the abnormal compression or concentration of the molten mass during the period of superheating and also to the subsequent enormous force of contraction due to the sudden chilling of its surface, the sound-record molded by my process is much denser 90 and harder on the surface than in case of an ordinary record made in the usual manner. It is, so to speak, "case-hardened" or tempered. Further, inasmuch as this symmetrical chilling effect takes place from the exterior of the mold and its casting I have discovered that with the composition at present employed (which is a mixture of two ingredients, as stearic acid and ceresin, both the

hardness and the melting-point or solidifying-point of one ingredient being higher than those of the other) the first effect of this sudden exterior chilling is an initial reduction of 5 the temperature to a point below the solidifying-point of the harder ingredient, which is thereupon converted into a thin shell or film, while the softer ingredient (still remaining liquid) is consequently forced inward. The 10 result is as already indicated—viz., a casting whose exterior surface is much harder and denser than its mass, though the gradation is so gradual and imperceptible that there is no line of separation that might cause the outer 15 casting to break off or the inner to shrink away.

Instead of admitting steam after the wax has been poured into the mold it may be admitted simultaneously or beforehand, as the object to be accomplished is the superheating 20 of the molten mass and the maintaining of that heat. It is obvious that other means may be employed for superheating the material while in the mold.

Among the superior advantages of my case-hardened record so produced are that the mass 25 being denser is less liable to be affected by changes of temperature and moisture and that being harder it is not so readily worn out by the action of a reproducing-stylus. Besides, while it would be difficult to engrave 30 a satisfactory original sound-record upon a surface as hard as that produced by my process, yet by this process a sound-record equally as good as an original record is readily and 35 cheaply produced in a more durable condition.

Of course I do not limit myself either to a cylindrical sound-record or to one of the type characterized by vertical irregularities, since 40 the spirit of my invention consists in maintaining the molten wax (while in connection with its matrix) in a superheated condition and in then suddenly and symmetrically chilling it.

45 The record produced by the process herein described gives improved results in reproduction and is more durable than records made by direct engraving. In the latter the surface over which the reproducer-point rubs 50 in reproducing is made by a cutting or scraping instrument having a blunt edge. When this surface is examined under a magnifying-glass, it is seen to be roughly broken, the molecules of wax having been disturbed and

their adhesion to one another weakened. 55 The reproducing-stylus rubbing over such a surface detaches these projecting particles, further roughening the surface, and causing scratching sounds in the reproduction. On the other hand, the surface of the molded 60 record being formed by the cooling of melted particles strongly adherent one to another offers far greater resistance to roughening by the reproducer. Such records therefore have longer life than those made in the ordinary way. 65

The improved sound-record resulting from the process herein described is claimed in a divisional application filed May 21, 1901, Serial No. 61,267. 70

Having thus described my invention, I claim—

1. The process of molding sound-records which consists in filling a suitable matrix with a suitable composition, maintaining the 75 same for a length of time in a superheated condition, and then suddenly and symmetrically chilling it, substantially as described.

2. The process of making a sound-record, which consists in pouring a suitable melted 80 material into a suitable matrix-mold, then admitting steam into a jacket surrounding said matrix and continuing this step until the said material has become limpid and impurities are driven off and the said material 85 forced into intimate contact with its matrix, then allowing the steam to escape and admitting cold water into the jacket whereby the said material is suddenly and symmetrically chilled from its exterior surface next 90 its matrix, substantially as and for the purpose set forth.

3. The process of molding sound-records which consists in filling a suitable matrix with a suitable material and maintaining the 95 same for a length of time in a superheated condition, and then suddenly and symmetrically chilling the same from the exterior inward, substantially as and for the purpose described. 100

In testimony whereof I have signed this specification in the presence of two subscribing witnesses.

THOMAS H. MACDONALD.

Witnesses:

W. R. MILLER,  
W. C. LEWIS.